

Patented May 29, 1928.

1,671,952

## UNITED STATES PATENT OFFICE.

LEWIS R. BRINK, OF CHICAGO, ILLINOIS, ASSIGNOR TO BARNHABT BROTHERS & SPINDLER, OF CHICAGO, ILLINOIS, A CORPORATION OF NEW JERSEY.

### METAL ALLOY.

No Drawing.

Application filed June 7, 1926. Serial No. 114,102.

My invention relates to metal alloys.

One of the objects of the invention is to provide a new and advantageous metal alloy.

Another object of the invention is to provide a metal alloy particularly adapted for use for printing types.

In accordance with my invention I provide a metal alloy having such elements or constituents that it will be especially well adapted for printing types which may be formed or made on die casting machines, in other words a metal alloy especially adapted for die cast type.

The metal alloy embodying my invention is preferably composed of about the following constituents:

|           | Per cent.        |
|-----------|------------------|
| Aluminum  | approximately 90 |
| Copper    | approximately 5  |
| 20 Nickel | approximately 5  |
| Total     | 100              |

An alloy embodying these elements or constituents may be combined or united in the manner usual or customary in forming metal 25 alloys for die casting.

The alloy thus composed has the requisite hardness and also the requisite toughness and durability to permit die casting of types and to form types which will be both durable to 30 permit long and hard usage and also accurate in point of size so as to insure proper printing.

It will be understood that changes and modifications may be made without departing from the spirit of the invention.

What I claim is:

A metal alloy consisting of approximately 90 per cent aluminum, approximately 5 per cent copper and approximately 5 per cent 40 nickel.

In witness whereof, I hereunto subscribe my name this 28th day of May A. D., 1926.

LEWIS R. BRINK.